

1

2,977,301

## WIDE-TEMPERATURE RANGE GREASES

Charles R. Bergen, Schenectady, N.Y., and William P. Scott, Richard M. Tillman, and Warren W. Woods, Ponca City, Okla., assignors to Continental Oil Company, Ponca City, Okla., a corporation of Delaware

No Drawing. Filed Aug. 21, 1958, Ser. No. 756,302

22 Claims. (Cl. 252—18)

The present invention relates to improved wide-temperature range greases and, more particularly, relates to such greases containing an agent for reducing extreme thixotropy therein.

Greases prepared by the use of the normal soap-forming ingredients, such as the acids derived from animal fats or vegetable oils, exhibit phase changes with increasing temperature up to a point at which the soap dissolves or at least forms a colloidal dispersion in the lubricating oil base with consequent loss of mechanical structure responsible for grease-like properties. Furthermore, these greases generally do not reform spontaneously upon cooling. As a result, such greases are unsuitable for use in the lubrication of bearings operated at elevated temperatures, such as those used in certain aircraft mechanisms and the like.

Several methods of preparing wide-temperature range greases have been proposed in the prior art. One proposal incorporates certain salts of aromatic acids in the grease composition such as sodium benzoate, which apparently forms complexes with the normal soap-forming acids. While these additives impart heat stability to the resulting grease, it is necessary to heat such grease compositions during the process of manufacture to a temperature of at least 500 to 600° F. This is a disadvantage because temperatures in this range involve fire hazards and promote oxidative degradation of the oil carrier. Another method heretofore proposed for the preparation of heat-stable greases involves the formation of an inorganic hydrogel and subsequently replacing the interstitial water contained in the gel with an oleaginous liquid vehicle. Two procedures have been suggested for the replacement of the interstitial water. In one, an aerogel is first formed by displacing the water with a solvent which is soluble in both water and oil. In the second procedure the hydrogel is heated in the presence of a surface-active agent dissolved in an oleaginous liquid vehicle; U.S. Patent 2,625,508 to Fred H. Stross describes this procedure. Whichever procedure is used, several disadvantages are inherent in the process, as, for example, a hydrogel is bulky and difficult to handle, the gel must be washed to remove salts, and hydrogels contain a large amount of water which must be removed.

In order to prepare greases which are satisfactory over the temperature range of —100° F. to above 450° F., it is necessary to use as base fluids those materials which in themselves have a satisfactory viscosity-temperature relationship over the temperatures involved. At the present time this requirement limits the base fluids to the synthetic types.

Normal thixotropy is an essential characteristic of greases; however, in the extreme, thixotropy causes an undesirable hardening during storage; and under working conditions (such as exist in a bearing), an intolerable softening occurs, allowing the grease to escape from the rubbing surfaces. It is desirable to have a grease which has relatively the same penetration under extreme work-

2

ing conditions as under light conditions. This property is known as work stability. While theoretically the terms "extreme thixotropy" and "work stability" are not the same, for all practical purposes in this disclosure they are considered equivalent.

It is an object of the present invention to provide improved grease compositions operable over a wide temperature range. It is still another object of the present invention to provide such improved grease compositions which do not exhibit extreme thixotropy. Other objects will become apparent as the invention is hereinafter more thoroughly described.

Broadly stated, the improved grease compositions of the present invention comprise a major amount of an oleaginous vehicle, a minor amount of a grease-forming agent, said grease-forming agent consisting of a colloidal dispersion of both calcium carbonate and the reaction product of calcium carbonate and a low molecular weight polycarboxylic acid in the presence of a metal sulfonate, and a minor amount of an agent for reducing extreme thixotropy in said grease compositions.

Materials which are suitable for use as an oleaginous vehicle, or base fluid, include the following:

25 Aliphatic diesters:

Di-isooctyl azelate  
Di-2-ethylhexyl sebacate  
Di-2-ethylhexyl azelate  
Di-2-ethylhexyl adipate  
Di-2-ethylpropyl azelate  
Di-2-ethylbutyl azelate

Polyesters:

Pentaerythritol tetracaproate

Silicate esters:

35 Hexa-(2-ethyl butoxy) disiloxane  
Hexa-(2-ethyl hexoxy) disiloxane

While at the present time synthetic fluids are the preferred oleaginous vehicle, this invention is not limited thereto. Other materials which have the necessary viscosity-temperature relationship over the temperature range desired could fall within the spirit and scope of this invention.

The grease-forming agent of the present invention is prepared by forming a colloidal dispersion of calcium carbonate in calcium sulfonate and reacting therewith an appropriate amount of a low-molecular weight polycarboxylic acid. If desired, the reaction may take place in the presence of an amount of the base fluid, wherein the grease-forming agent is formed *in situ*.

The colloidal dispersion of calcium carbonate in calcium sulfonate is prepared as follows:

(a) a methanolic solution of calcium sulfhydrate is prepared,

55 (b) a solution is then prepared containing the methanolic calcium sulfhydrate and a sulfonic acid solution in benzene as a solvent,

(c) the solution is blown with carbon dioxide,

(d) the desired base fluid is added and the volatile solvents removed.

The preparation of this colloidal dispersion of calcium carbonate in calcium sulfonate is disclosed also by Robert L. Carlyle in S.N. 629,229, filed December 19, 1956, now U.S. Patent No. 2,937,991.

65 The calcium sulfhydrate is prepared by adding calcium oxide, calcium hydroxide, or the hydrates of calcium hydroxide, to an alcohol and blowing with hydrogen sulfide. Suitable alcohols include those of the aliphatic primary series having from 1 to 6 carbon atoms. Of these alcohols, methanol is preferred. The solution is then filtered to remove impurities.

Any of the sulfonic acids, or sulfonates, normally used in the manufacture of lubricating oil additives may be used as the dispersing agent in the grease-forming agent. Examples of these materials would include the mahogany sulfonates, diwaxbenzene sulfonates, dinonylnaphthalene sulfonates and postdodecylbenzene sulfonic acid. Post-dodecylbenzene is a by-product of the manufacture of dodecylbenzene, being the "bottoms" after distilling the dodecylbenzene and postdodecylbenzene overhead. This material is also known as stripped postdodecylbenzene, the terms being synonymous in this disclosure. For the sake of simplicity, postdodecylbenzene is often referred to as PDB, and will be so used in this disclosure.

Postdodecylbenzene consists of monoalkylbenzenes and dialkylbenzenes in the approximate mole ratio of 2 to 3. Its typical physical properties are as follows:

|                            |                  |
|----------------------------|------------------|
| Specific gravity at 38° C. | 0.8649           |
| Average molecular weight   | 385              |
| Percent sulfonatable       | 88               |
| A.S.T.M.—D-158-Engler:     |                  |
| I.B.P.                     | ° F. 647         |
| 5                          | ° F. 682         |
| 50                         | ° F. 715         |
| 90                         | ° F. 760         |
| 95                         | ° F. 775         |
| F.B.P.                     | ° F. 779         |
| Refractive index at 23° C. | 1.4900           |
| Viscosity at:              |                  |
| -10° C.                    | centipoises 2800 |
| 20                         | do 280           |
| 40                         | do 78            |
| 80                         | do 78            |
| Aniline point              | ° C. 69          |
| Pour point                 | ° F. -25         |

Suitable low-molecular weight polycarboxylic acids for use in this invention include the following:

3-methyl glutaric acid  
Itaconic acid  
Pyromellitic acid  
2-methyl adipic acid  
3-tertiary butyl adipic acid  
3-tertiary amyl adipic acid  
Octyl adipic acid  
Furoic acid  
Mercapto succinic acid  
2,2-dibromo succinic acid  
5-methyl-4-cyclohexane-1,2-dicarboxylic acid  
(m-Phenylenedioxy) diacetic acid  
Benzylmalonic acid  
Terephthalic acid  
Thiodiglycolic acid

Of these, 3-methyl glutaric acid is preferred.

Two types of materials have been found to be suitable for use as agents for reducing extreme thixotropy. These are the methacrylate ester co-polymers and the silicone polymers. The methacrylate ester co-polymers used in this invention have the formula



where R is a mixture of alkyl groups containing from 4 to 20 carbon atoms and n is a number providing a molecular weight of the co-polymer of about 15,000 to 40,000. Commercial methacrylate ester co-polymers which may be used are those sold under the "Acryloid" trade name. Specific examples of these materials include the following: Acryloid 618, Acryloid 710, Acryloid 763, and Acryloid 794.

Suitable silicone polymers which may be used include the polymethylsiloxanes, phenyl substituted polymethylsiloxanes, and chlorinated polysiloxanes. Suitable commercially available materials are those sold under the

"DC" trade name by Dow-Corning, as for example "DC 510" (phenyl substituted polymethylsiloxane), "DC 200" (polymethyl siloxane), and "DC 371" (poly-methylethyl siloxane). Other suitable commercially available materials are those sold by General Electric, for example "SF-81" and "SF-96," and by Union Carbide and Carbon, for example, "L-45" and "L-522." These materials are available in various viscosity or molecular weight grades, such as 50 centistokes, etc.

In order to disclose more clearly the nature of the present invention and the advantages thereof, reference will hereinafter be made to certain specific embodiments which illustrate the flexibility of the herein described process. It should be clearly understood, however, that this is done solely by way of example and is not to be construed as a limitation upon the spirit and scope of the appended claims.

#### EXAMPLE I

##### Preparation of colloidal dispersion of calcium carbonate in calcium sulfonate

A methanolic solution of calcium sulfhydride was prepared as previously described.

##### Materials used:

|                                                                                                    |              |
|----------------------------------------------------------------------------------------------------|--------------|
| PDB sulfonic acid in naphtha (0.787 milli-equivalents per gram—total acidity; 28.7 percent active) | grams 2926.8 |
| Benzene (solvent)                                                                                  | ml 3000      |
| Calcium sulfhydride in methanol (4.2 milli-equivalents Ca per gram)                                | grams 1641   |
| Di-2-ethyl hexyl azelate (base fluid)                                                              | do 1607.8    |

Procedure: The PDB sulfonic acid, calcium sulfhydride and benzene were added to a suitable reaction vessel. The mixture was blown with carbon dioxide while stirring until essentially all H<sub>2</sub>S had been expelled. The di-2-ethyl hexyl azelate was added to the reaction vessel. The solvents were removed by heating to 150° C. while blowing with carbon dioxide.

This material had a theoretical composition as follows:

|                          | Weight percent |
|--------------------------|----------------|
| CaCO <sub>3</sub>        | 8.4            |
| Ca PDB sulfonate         | 32.5           |
| Di-2-ethyl hexyl azelate | 59.1           |

The material had an actual base number (acetic) of 102, as compared to a theoretical one of 94.4.

#### EXAMPLE II

##### Preparation of base grease

##### Materials used:

A

|                                          |           |
|------------------------------------------|-----------|
| Calcium carbonate dispersion (Example I) | grams 992 |
| Di-2-ethyl hexyl azelate                 | do 762    |
| Benzene                                  | ml 908    |

B

|                        |             |
|------------------------|-------------|
| 3-methyl glutaric acid | grams 105.2 |
| Benzene                | ml 908      |
| Acetone                | ml 908      |

Procedure: The Group A materials were added to a suitable reaction vessel. A solution was prepared of Group B materials, and this was added to the reaction vessel while stirring the contents. The solvents were removed by heating to 195° C. while stirring and blowing with nitrogen.

This grease had a theoretical composition as follows:

|                            | Weight percent |
|----------------------------|----------------|
| Ca PDB sulfonate           | 11.54          |
| Calcium-3-methyl glutarate | 7.3            |
| Calcium carbonate          | 0.7            |
| Di-2-ethyl hexyl azelate   | 80.46          |

5  
EXAMPLE III

The product of Example II was found to exhibit extreme thixotropy. Methacrylate ester co-polymers in various amounts and of various compositions were added to this base grease. This was done simply by adding a known percentage of methacrylate ester co-polymers to the base grease and homogenizing the resulting product. The results of the use of the methacrylate ester co-polymers is shown in Table I.

TABLE I  
*Use of agents for reducing extreme thixotropy*

| Polymer                               | Percent Addition | Penetration,<br>60 Strokes | Penetration,<br>3,000 Strokes |
|---------------------------------------|------------------|----------------------------|-------------------------------|
| Base Grease (Example II) <sup>1</sup> |                  | Fluid                      | 345                           |
| Base Grease+Acryloid 618              | 5                | 346                        | 345                           |
| Base Grease+Acryloid 710              | 5                | 325                        | 330                           |
| Base Grease+Acryloid 710              | 10               | 305                        | 320                           |
| Base Grease+Acryloid 763              | 5                | 345                        | 350                           |
| Base Grease+Acryloid 794              | 5                | 350                        | 355                           |

<sup>1</sup> Unworked penetration=280.

<sup>2</sup> A.S.T.M. Method D217.

EXAMPLE IV  
*Preparation of base grease*

Materials used:

A

Calcium carbonate dispersion (109.5 g. CaCO<sub>3</sub>, 423.7 g. Ca PDB sulfonate, balance di-2-ethyl hexyl azelate) grams 1304  
Di-2-ethyl hexyl azelate do 1281  
Benzene ml 1361

B

Acetone solution of 3-methyl glutaric acid (1 ml.=0.2 g. acid) ml 683  
Acetone ml 478  
Benzene ml 1361

Procedure: The same procedure as used in Example II was employed here.

This grease had a theoretical composition as follows:

|                          | Weight percent |
|--------------------------|----------------|
| Ca PDB sulfonate         | 15.91          |
| Ca-3-methyl glutarate    | 6.46           |
| CaCO <sub>3</sub>        | 0.6            |
| Di-2-ethyl hexyl azelate | 77.03          |

EXAMPLE V

The product of Example IV was found to have extreme thixotropy. Varying amounts of a phenyl substituted polymethyl-siloxane ("DC-510"—50 c.s. grade) were added to the base grease. Again, this was done simply by adding a known percentage and homogenizing the resulting product. Penetration data for this example is shown in Table II.

TABLE II  
*Use of silicone polymer for reducing extreme thixotropy*

| Base Grease | Percent Addition of Silicone Fluid | Penetration Strokes <sup>1</sup> |       |        |         |
|-------------|------------------------------------|----------------------------------|-------|--------|---------|
|             |                                    | 60                               | 3,000 | 10,000 | 100,000 |
| Example IV  | 0                                  | 265                              | 355   | 355    | Fluid   |
| Do          | 1                                  | 300                              | 370   | 370    | Fluid   |
| Do          | 3                                  | 290                              | 320   | 325    | 340     |
| Do          | 6                                  | 280                              | 305   | 305    | 310     |
| Do          | 9                                  | 280                              | 290   | 300    | 305     |
| Do          | 12                                 | 275                              | 290   | 305    | 305     |

<sup>1</sup> A.S.T.M. Method D217.

6  
EXAMPLE VI

*Preparation of grease containing silicone polymer*

Materials used:

|    |                                                                                              |  |
|----|----------------------------------------------------------------------------------------------|--|
| 5  | Calcium carbonate dispersion (8.5% CaCO <sub>3</sub> , 26.65% Ca PDB sulfonate) grams 1086.4 |  |
| 10 | Di-2-ethyl hexyl azelate do 1116.3                                                           |  |
| 15 | Benzene ml 1134                                                                              |  |

A

|                                                                                              |  |
|----------------------------------------------------------------------------------------------|--|
| Calcium carbonate dispersion (8.5% CaCO <sub>3</sub> , 26.65% Ca PDB sulfonate) grams 1086.4 |  |
| Di-2-ethyl hexyl azelate do 1116.3                                                           |  |
| Benzene ml 1134                                                                              |  |

B

|                                                                   |  |
|-------------------------------------------------------------------|--|
| Acetone solution of 3-methyl glutaric acid (113.9 g. acid) ml 570 |  |
| Acetone ml 565                                                    |  |
| Benzene ml 1134                                                   |  |

C

|                              |  |
|------------------------------|--|
| DC-510 (50 c.s.) grams 197.2 |  |
|------------------------------|--|

Procedure: The Group A materials were added to a suitable reaction vessel. A solution was prepared of Group B materials, and this was added to the reaction vessel while stirring the contents. The solvents were removed by heating to 150° C. At this stage the DC-510 was added. (This is 8 percent by weight of theoretical product.) The product was stirred and heated to 195° C. while blowing dry air over the grease.

This grease had a theoretical composition as follows:

|                          | Weight percent |
|--------------------------|----------------|
| Ca PDB sulfonate         | 11.74          |
| Ca-3-methyl glutarate    | 5.82           |
| CaCO <sub>3</sub>        | 0.56           |
| Di-2-ethyl hexyl azelate | 73.88          |
| DC-510                   | 8.0            |

The penetration data on this grease is shown in Table III. An additional amount of silicone polymer was added to a portion of the product. This was done simply by adding a known amount and homogenizing the resulting product. Penetration data for this example is shown in Table III.

TABLE III  
*Use of silicone polymer as work stability improver*

| 45        | Base Grease | Percent Addition of Silicone Fluid | Penetration Strokes <sup>1</sup> |       |
|-----------|-------------|------------------------------------|----------------------------------|-------|
|           |             |                                    | 60                               | 3,000 |
| Example V |             | 8                                  | 310                              | 360   |
| Do        |             | 15                                 | 325                              | 325   |

<sup>1</sup> A.S.T.M. Method D217.

The data presented in Table I indicate clearly that the use of methacrylate ester co-polymers reduces extreme thixotropy and improves the work stability of these particular greases. The data in Table II indicate that silicone polymers also function very well for this purpose. Example VI and the resulting data in Table III have been included to demonstrate that silicone polymers function as a work stability agent for this grease. The grease of Example VI differs from the grease of Example IV primarily in the amount of sulfonate present.

While particular embodiments of the invention have been described, it will be understood, of course, that the invention is not limited thereto, since many modifications may be made; and it is, therefore, contemplated to cover by the appended claims any such modifications as fall within the true spirit and scope of the invention.

The invention having thus been described, what is claimed and desired to be secured by Letters Patent is:

1. A grease composition comprising a major amount of a synthetic lubricant selected from the group consisting of aliphatic diesters, polyesters, and silicate esters, a minor amount of a grease-forming agent, said grease-forming agent consisting of a colloidal dispersion in an

oil-soluble metal sulfonate of both calcium carbonate and the reaction product of calcium carbonate and a low molecular weight polycarboxylic acid selected from the group consisting of 3-methyl glutaric acid, itaconic acid, pyromellitic acid, 2-methyl adipic acid, 3-tertiary butyl adipic acid, 3-tertiary amyl adipic acid, octyl adipic acid, furoic acid, mercapto succinic acid, 2,2-dibromo succinic acid, 5-methyl-4-cyclohexane-1,2-dicarboxylic acid, (m-phenylenedioxy) diacetic acid, benzylmalonic acid, terephthalic acid, and thiodiglycolic acid in the presence of an oil-soluble metal sulfonate, wherein the amount of said acid is equivalent to that which varies from 37 to 85 percent of that theoretically required for neutralization of said calcium carbonate originally present, and a minor amount of an agent for reducing extreme thixotropy in said grease composition, said agent being selected from the group consisting of methacrylate ester co-polymers having molecular weights in the range of 15,000 to 40,000 and silicone polymers.

2. A grease composition as defined in claim 1, wherein the synthetic lubricant is an aliphatic diester.

3. A grease composition as defined in claim 1 wherein the synthetic lubricant is an aliphatic polyester.

4. A grease composition as defined in claim 1 wherein the synthetic lubricant is an aliphatic silicate ester.

5. A grease composition as defined in claim 1 wherein the low molecular weight polycarboxylic acid is 3-methyl glutaric acid.

6. A grease composition comprising a major amount of an aliphatic diester, a minor amount of a grease-forming agent, said grease-forming agent consisting of a colloidal dispersion in an oil-soluble metal sulfonate of both calcium carbonate and 3-methyl glutaric acid in the presence of an oil-soluble metal sulfonate, wherein the amount of said acid is equivalent to that which varies from 37 to 85 percent of that theoretically required for neutralization of said calcium carbonate originally present, and a minor amount of an agent for reducing extreme thixotropy in said grease composition, said agent being selected from the group consisting of methacrylate ester co-polymers having molecular weights in the range of 15,000 to 40,000 and silicone polymers.

7. A grease composition as defined in claim 2, wherein the agent for reducing extreme thixotropy in said grease composition is a methacrylate ester co-polymer having a molecular weight in the range of 15,000 to 40,000.

8. A grease composition as defined in claim 2, wherein the agent for reducing extreme thixotropy in said grease composition is a polymethylsiloxane.

9. A grease composition as defined in claim 2, wherein the agent for reducing extreme thixotropy in said grease composition is a phenyl substituted polymethylsiloxane.

10. A grease composition as defined in claim 2, wherein the agent for reducing extreme thixotropy in said grease composition is a chlorinated polysiloxane.

11. A grease composition as defined in claim 3, where-

in the agent for reducing extreme thixotropy in said grease composition is a methacrylate ester co-polymer having a molecular weight in the range of 15,000 to 40,000.

12. A grease composition as defined in claim 3, wherein the agent for reducing extreme thixotropy in said grease composition is a polymethylsiloxane.

13. A grease composition as defined in claim 3, wherein the agent for reducing extreme thixotropy in said grease composition is a phenyl substituted polymethylsiloxane.

14. A grease composition as defined in claim 3, wherein the agent for reducing extreme thixotropy in said grease composition is a chlorinated polysiloxane.

15. A grease composition as defined in claim 4, wherein the agent for reducing extreme thixotropy in said grease composition is a methacrylate ester co-polymer having a molecular weight in the range of 15,000 to 40,000.

16. A grease composition as defined in claim 4, wherein the agent for reducing extreme thixotropy in said grease composition is a polymethylsiloxane.

17. A grease composition as defined in claim 4, wherein the agent for reducing extreme thixotropy in said grease composition is a phenyl substituted polymethylsiloxane.

18. A grease composition as defined in claim 4, wherein the agent for reducing extreme thixotropy in said grease composition is a chlorinated polysiloxane.

19. A grease composition as defined in claim 4, wherein the agent for reducing extreme thixotropy in said grease composition is a methacrylate ester co-polymer having a molecular weight in the range of 15,000 to 40,000.

20. A grease composition as defined in claim 6, wherein the agent for reducing extreme thixotropy in said grease composition is a polymethylsiloxane.

21. A grease composition as defined in claim 6, wherein the agent for reducing extreme thixotropy in said grease composition is a phenyl substituted polymethylsiloxane.

22. A grease composition as defined in claim 6, wherein the agent for reducing extreme thixotropy in said grease composition is a chlorinated polysiloxane.

#### References Cited in the file of this patent

#### UNITED STATES PATENTS

|           |                   |               |
|-----------|-------------------|---------------|
| 2,349,817 | Farrington et al. | May 30, 1944  |
| 2,363,514 | Farrington et al. | Nov. 28, 1944 |
| 2,528,373 | Knowles et al.    | Oct. 31, 1950 |
| 2,616,904 | Asseff et al.     | Nov. 4, 1952  |

#### OTHER REFERENCES

55 "The Manufacture and Application of Lubricating Greases," Boner-Reinhold Pub. Corp., N.Y., 1954, pp. 443 and 445.